

1

2,872,307

## THORIUM-CARBON ALLOYS

Harley A. Wilhelm and Robert E. Rundle, Ames, Iowa, assignors to the United States of America as represented by the United States Atomic Energy Commission

No Drawing. Application February 25, 1949  
Serial No. 78,477

2 Claims. (Cl. 75—122.7)

This invention relates to alloys of thorium and carbon and more particularly to thorium-carbon alloys having a low carbon content.

An object of this invention is to provide a thorium-carbon alloy having a selected low carbon content and preferably a thorium-carbon alloy containing the percentage of carbon within those certain limits which will impart to the cast alloy properties superior to those found in pure thorium metal.

A further object of this invention is to provide a new composition of matter, namely, thorium monocarbide (ThC).

A further object of this invention is to provide a thorium-carbon alloy wherein the carbon present as a solid solution in thorium metal is present in the form of the compound, thorium monocarbide.

Other objects and advantages of this invention will be readily apparent from the following description of the preferred embodiments of this invention.

The compositions of matter comprising the subject matter of this invention possess properties which make them useful in processes involving nuclear bombardment under conditions peculiar to those found in chain-reacting piles. The particular carbon content found in these compositions of matter imparts to them the properties of increased hardness and resistance to corrosion from contact with hot aqueous solutions.

In accordance with this invention, carbon is incorporated into thorium metal to produce the compound, thorium monocarbide, and mixtures consisting of thorium metal and thorium monocarbide. The monocarbide and mixtures of thorium metal with thorium monocarbide possess greater hardness and resistance to corrosion than thorium metal alone.

The thorium alloy comprising the subject matter of this invention contains a carbon content between 0.1 and 4.9% by weight carbon. Generally, the hardness values increase directly with the increase in carbon content, and those thorium-carbon alloys containing between 0.1 and 2% by weight carbon are preferred. Alloys containing 0.1 to 0.5% carbon are especially preferred.

The alloys or compositions of matter comprising this invention are prepared by heating thorium metal with carbon at a temperature above the melting point of thorium, for example, at 1800 to 2000° C. in an inert refractory crucible. The reaction may be carried out in a vacuum or in the presence of an inert gas, such as argon and helium, to prevent thorium oxide formation.

When using a graphite vessel in the casting of thorium, the carbon of a graphite vessel reacts with thorium in sufficient quantity to introduce less than 0.1% carbon which occurs as carbide in the metal both as grain boundary and intergranular inclusions. However, in a method of preparing the alloys of this invention pure thorium is heated for a prolonged period of time above its melting point in a graphite crucible whereby thorium and graphite react to produce the alloys. The carbon

2

content of the alloy is determined by the time of heating thorium in the crucible for a particular temperature. The amount of carbon thereby introduced may be varied between 0.1 and 4.9% by weight. Thorium-carbon alloys of this invention having low carbon contents, such as 0.1 to 2%, may be prepared by fusing thorium with an appropriate amount of carbon in a crucible of a refractory oxide, such as thoria, using an atomic hydrogen arc.

10 After the fused alloy is obtained by any of the foregoing methods, it may be water-quenched or furnace-cooled in an inert atmosphere from the reaction temperature.

We have discovered that cast alloys of thorium containing between 0.1 and 0.5% by weight carbon are more resistant to water corrosion than pure thorium metal. The extent of corrosion resistance in these alloys was determined by subjecting samples to an autoclave treatment. Specimens of the cast alloy were prepared by hand polishing with various grades of emery paper, finishing with No. 1 grit paper and washing with acetone after hand polishing to remove emery, dirt, and particles. The surface area was measured after rewashing in acetone and the samples were weighed. The specimens were then immersed in boiled distilled water contained in a 400-cc. beaker which was then covered with a Petri dish and heated in an autoclave by steam at 178° C. under a pressure of 125 lbs. per square inch. At certain intervals, the specimens were removed from the water, dried with acetone, weighed, and placed back in the water in the autoclave for continued treatment. Table I summarizes the extent of corrosion observed in a thorium alloy containing 0.3% carbon and in pure thorium metal.

TABLE I

| Time in Test, hrs. | Total Wt. Change, mg./cm. <sup>2</sup> /hr. |         |
|--------------------|---------------------------------------------|---------|
|                    | Th alloy containing 0.3% C                  | Pure Th |
| 40                 |                                             |         |
| 19.2               | -0.0047                                     | +0.0245 |
| 96                 | -0.0017                                     | -0.004  |
| 192                | -0.0036                                     | -0.064  |
| 286                |                                             | -0.13   |
| 384                | -0.0010                                     | -0.246  |
| 768                | -0.0009                                     | -0.453  |

The data indicate that the loss in weight due to corrosion of pure thorium is much greater than the loss of the thorium alloy.

When alloys of the present invention are water-quenched from elevated temperatures, e. g., 1100° C., the hardness of the alloy is determined by the carbon content. By increasing the carbon content the hardness of the alloy increases. However, it was found that by subsequent annealing of these water-quenched alloys at elevated temperatures, such as 700, 800, 900, and 1000° C., for six hours and followed by furnace-cooling, the alloys containing greater than 0.5% carbon lost substantial amounts of their hardness. In all cases these alloys still had hardness values greater than alloys containing less than 0.5% carbon. The latter alloys exhibited substantially no change in hardness when subjected to this annealing treatment and they are accordingly alloys of relatively permanent hardness.

Apparently, carbon is soluble in thorium metal as a solid solution of thorium monocarbide. At 900° C., carbon is soluble in thorium to the extent of less than 0.12%. At 1000° C. the solubility limit for carbon in thorium is between 0.32 and 0.44% carbon, while at 1100° C., between 0.44 and 0.74% by weight carbon is

soluble in thorium metal. These values expressed in percent by weight of thorium monocarbide would be:

At 900° C. 2.44% ThC  
At 1000° C. from 6.5 to 8.9% ThC  
At 1100° C. from 8.9 to 15% ThC

X-ray diffraction studies were also made on the compositions of matter which constitute the subject of this invention. All quenched samples were examined by X-ray diffraction, which revealed the presence of distinct thorium and thorium-carbon phases. The thorium monocarbide phase is identified by a face-centered cubic NaCl-type structure having a lattice parameter  $a_0=5.29$  Å. Determinations of lattice parameter were determined by obtaining a back reflection pattern from a polished surface of the alloy sample. The lattice parameter for pure thorium metal is  $5.074\pm0.002$  Å. at 20° C., which value increases directly with an increase in the percent carbon present in the sample and the temperature at which the alloy is heated and subsequently water-quenched. Such data indicate that the presence of carbon expands the crystal lattice structure of metal and furnishes additional evidence for the solid solubility of carbon in thorium.

*Example I*

A sample of thorium metal was fused in an atomic hydrogen arc in the presence of carbon. The resultant product was ground and polished and an average hardness of 53 on the Rockwell A scale was measured. X-ray data revealed the presence of three phases, namely, thorium metal, thorium dioxide, and thorium monocarbide. Chemical analysis of this product show 0.34% carbon and 90% thorium. Photomicrographs showed the presence of a dendritic monocarbide pattern.

*Example II*

A sample of thorium metal was fused in a graphite crucible and the resultant product was found to contain 1.2% carbon and 98.5% total thorium (84.8% free thorium as determined by hydrogen evolution). The X-ray diffraction pattern showed a lattice parameter for thorium  $a_0=5.094$  Å. and the thorium monocarbide lattice parameter 5.28 Å., the monocarbide phase being a face-centered NaCl-type structure. The average hardness was 62.1 on the Rockwell A scale which was equivalent to approximately 100 on the Rockwell B scale. Examination of the microstructure showed carbide in the grain boundaries and some distribution of carbide throughout the crystal planes.

*Example III*

A thorium-zinc metal biscuit was heated in an induction furnace to a temperature of 1850° C. under high vacuum in a graphite crucible in order to distill off the zinc impurity. When the vapor pressure had dropped to a low value, purified argon was introduced to prevent surface oxidation of the metal while cooling it.

The resultant metal contained 99% free thorium, 99.7% total thorium and 0.09% carbon.

A sample of this thorium metal, weighing 196.5 g., was heated in a beryllium oxide crucible with 0.492 g. of carbon to a temperature of 1850° C. for fifteen minutes and subsequently water-quenched from this temperature. The average hardness value of the resultant thorium-carbon alloy was 93.9 on the Rockwell B scale. Chemical analysis showed 0.36% carbon. The X-ray diffraction pattern for the starting material showed a lattice parameter  $a_0=5.0835\pm0.0004$  Å., while the lattice parameter for the thorium-carbon product alloy was  $a_0=5.0887\pm0.0005$  Å.

*Example IV*

The pure thorium metal used in this experiment was prepared by the vacuum distillation of zinc from a zinc-thorium alloy as in Example III.

One hundred sixty-eight grams of the dezinced thorium metal containing 0.04% carbon was heated with 0.88 g. of carbon in a graphite crucible lined with beryllia to a temperature of 2000° C. The temperature was lowered by passing argon into the system and at 1850° C. the carbon crucible containing the sample was quenched in water. Average hardness values on the Rockwell B scale measured 92.4 and the product contained 0.59% by weight carbon. The lattice parameter of the starting material which contained 0.04% carbon is equal to  $a_0=5.0794\pm0.0006$  Å., while the product lattice parameter was  $a_0=5.094\pm0.0006$  Å.

The foregoing description presents the preferred embodiments of this invention in which are disclosed new and useful compositions of matter. Many alterations and changes, which will be apparent to those skilled in the art, may be made therein without departing from the spirit and scope of this invention as set forth in the appended claims.

What is claimed is:

1. A thorium-carbon alloy consisting essentially of 0.1 to 0.5% by weight carbon and thorium.
2. A binary thorium-carbon alloy consisting of thorium and about 0.3% by weight carbon.

References Cited in the file of this patent

FOREIGN PATENTS

542,410 Great Britain ----- Jan. 8, 1942

OTHER REFERENCES

50 Troost: Comptes Rendus, vol. 116, pp. 1229-1230 (1893).

Moissan et al.: Annales de Chimie et du Physique, Series 7, vol. 12, p. 432 (1897).

55 Mellor: Inorganic and Theoretical Chemistry, vol. 7, p. 210 (1927), publ. by Longmans, Green & Co., London.